

May 20, 1930.

P. H. LEDEBOER

1,759,753

METHOD FOR WORKING-UP IRON ORES IN A DIRECT WAY

Filed March 17, 1928



Inventor:  
P. Ledeboer,  
Deceased,  
H. E. M. G. Ledeboer,  
Administratrix,  
by  
Langmuir, Parry, Ward & Langmuir  
Att. '43.

Patented May 20, 1930

1,759,753

# UNITED STATES PATENT OFFICE

PIERRE HUGO LEDEBOER, DECEASED, LATE OF PARIS, FRANCE, BY ANTOINETTE ECHARIS MARIE GÉRARDIN LEDEBOER, ADMINISTRATRIX, OF PARIS, FRANCE, AS SIGNOR TO STAALSYNDICAAT DR. LEDEBOER II, OF THE HAGUE, NETHERLANDS

## METHOD FOR WORKING UP IRON ORES IN A DIRECT WAY

Application filed March 17, 1928, Serial No. 262,604, and in the Netherlands March 30, 1927.

This invention relates to the working up of iron ores in a direct way, that is without the use of a blast furnace. The direct way has been successful in so far that the reduction of the ore could be carried out satisfactorily in several ways, as for example in the manufacture of sponge iron. The iron being formed however is very inflammable and great difficulty is met in trying to separate it. For obtaining the iron in a molten state a heating source must be applied which under prevailing circumstances does not exert a detrimental oxidizing action and yet has the necessary temperature. To this purpose electrical heating in some way or other might be used, but in doing this any economical competition with the nowadays followed indirect methods (that is by the way of a blast furnace, making the half finished product raw iron) is precluded.

For this reason it has been tried to use the heat from a flame. As fuel, either pulverized coal or a combustible gas was used. In order to prevent the detrimental oxidizing action, it was found necessary in both cases to very incompletely burn the fuel. In this way the caloric value of the fuel was very uneconomically utilized, while moreover it is very doubtful whether even in applying the highest preheating applicable, it would be possible to obtain the necessary temperature.

It is already known to apply surface combustion, e. g. for heating furnaces.

Considering what has been previously attempted to effect economical and thorough extraction of iron from its ores and the disadvantages attending the carrying out of the old methods the present invention was conceived with the idea of evolving a method which may be carried out without the use of a blast furnace and enabling to obtain the iron in a molten state.

In the accompanying drawing is shown a schematic arrangement for carrying out the invention. In this view the furnace is indicated by the numeral 1 and the charge brought into a molten state by the heat from the combustion of fuel burned in the surface combustion burner 2 is indicated at 4. The combustion gas indicated at 3 passes over the

material that is treated as indicated by the arrows. The combustible mixture is admitted to the burner at 5 and the combustion gas is carried off at 6.

The invention therefore contemplates the method by which the iron ore is reduced and the iron is separated in a molten state and which method is characterized by the fact that as heating source for the melting process a combustion gas is applied which possesses the necessary temperature and practically contains no free oxygen and which combustion gas is obtained by means of a burner, acting according to the principle of surface combustion.

In general by means of surface combustion a combustion gas can be obtained which practically does not contain free oxygen and is formed by complete or nearly complete combustion, because this manner of combustion has the characteristic property of rendering possible a nearly complete combustion without an excess of oxygen (air).

In spite of the fact that the combustion is localized in a certain zone, the usual surface combustion burners furnish combustion gases having a temperature which is considerably lower than the theoretical combustion temperature.

In the present day development of the surface combustion however kinds of burners are constructed by means of which it is possible to obtain combustion gases having very high temperatures which more closely approach the theoretical combustion temperature. In spite of this fact it has been possible to prevent the withdrawal of the combustion zone, which was the cause of many failures in using former constructions in that it caused back-firing.

Particularly it has appeared that by means of burners constructed according to constructive principles of Lucke (Journal of Industrial and Engineering Chemistry 1913, page 801 and following pages) and of Essich (Stahl und Eisen 1921, page 228 and following pages) it is possible to produce combustion gases of a temperature high enough to melt even pure iron.

In this way, in using the principle of sur-

face combustion it is possible to obtain the combustion gas above mentioned as heating source for the melting process.

This newly introduced heating source possesses the necessary temperature for obtaining the iron in a molten state, and at the same time under prevailing circumstances does not exert a detrimental oxidizing action, thus enabling to separate the iron in a technically satisfactory way.

10 Furthermore this heating source is a very economical one, and enables the separating of the iron also in an economically satisfactory way.

15 What is claimed is:

16 A method for working up iron ores in a direct way by reducing the ore and by separating the iron in a molten state, characterized by the fact that as heating source for the melting process a combustion gas is applied, having the necessary temperature and practically containing no free oxygen, which combustion gas is obtained by means of a burner acting according to the principle of surface combustion.

25 In testimony whereof I have signed my name to this specification.

ANTINETTE EUCHARIS MARIE

GÉRARDIN LEDEBOER,

30 Administratrix of the estate of P. Ledeboer, deceased.